

United States Patent [19]  
Bressanelli

[11] 3,861,908  
[45] Jan. 21, 1975

[54] DUPLEX STAINLESS STEEL

[75] Inventor: Jerome P. Bressanelli, Scott Twp.,  
Allegheny County, Pa.

[73] Assignee: Crucible Inc., Pittsburgh, Pa.

[22] Filed: Aug. 20, 1973

[21] Appl. No.: 389,832

[52] U.S. Cl. .... 75/126 B, 75/126 C, 75/126 J,  
75/128 A, 75/128 N, 75/128 W

[51] Int. Cl. .... C22c 39/14

[58] Field of Search..... 75/126 A, 126 C, 128 A,  
75/126 J, 128 N, 128 W

[56] References Cited

UNITED STATES PATENTS

|           |         |                |          |
|-----------|---------|----------------|----------|
| 2,225,440 | 12/1940 | Becket.....    | 75/128 A |
| 2,357,885 | 9/1944  | Franks.....    | 75/126 B |
| 3,112,195 | 11/1963 | Souresny ..... | 75/126 B |

|           |         |              |            |
|-----------|---------|--------------|------------|
| 3,152,934 | 10/1964 | Lula.....    | 75/128 A   |
| 3,736,131 | 5/1973  | Espy .....   | 75/128 A X |
| 3,756,807 | 9/1973  | Hoshino..... | 75/128 A   |

Primary Examiner—C. Lovell  
Assistant Examiner—Arthur J. Steiner

[57] ABSTRACT

A duplex stainless steel having a good combination of hot workability, corrosion resistance and cold formability, said duplex stainless steel consisting essentially of, in weight percent, carbon 0.12 max., nitrogen 0.12 max., manganese 8 to 16, silicon 1.0 max., nickel 1.0 max., chromium 15 to 20, molybdenum 0.6 to 2.0, carbon + nitrogen 0.06 to 0.14 and the balance iron, the chromium equivalent of 13.5 to 16.0 in accordance with the formula:

Chromium equivalent in percent = %Cr + %Si + %Mo  
— %Ni — 30 (%C + %N).

3 Claims, 7 Drawing Figures

PATENTED JAN 21 1975

3,861,908

SHEET 1 OF 6



FIG. 1



FIG. 7

PATENTED JAN 21 1975

3,861,908

SHEET 2 OF 6

HEAT    %C + %N  
716        0.159

IE62    0.148

IE61    0.136

IE59    0.106

IE57    0.079



FIG. 2

PATENTED JAN 21 1975

3,861,908

SHEET 3 OF 6



FIG. 3

PATENTED JAN 21 1975

3,861,908

SHEET 4 OF 6



FIG. 4

PATENTED JAN 21 1975

3,861,908

SHEET 5 OF 6



FIG. 5

PATENTED JAN 21 1975

3,861,908

SHEET 6 OF 6



FIG. 6

## DUPLEX STAINLESS STEEL

For applications involving the manufacture of trim for motor vehicles, such as hubcaps, wheelcovers, bumpers, and the like, it is necessary to have a steel that possesses good hot-workability and yet may be cold formed to the desired trim configurations. In addition, during use in the corrosive environments incident to motor vehicle operation it is necessary that the steel provide good corrosion resistance. Further, in view of the increasing cost and scarcity of the element nickel, it is desirable to achieve these properties in an alloy that is essentially nickel free or where nickel is not present in more than what is typically termed a residual amount.

It is accordingly an object of the present invention to provide a substantially nickel-free, duplex stainless steel containing substantially equal amounts of ferrite and austenite after annealing at temperatures typically within the range of 1,850° to 2,050°F and characterized by good hot workability, good cold formability and corrosion resistance.

These and other objects of the invention, as well as a more complete understanding thereof may be obtained from the following description, specific examples and drawings, in which:

FIG. 1 is a graph showing the effect of carbon and nitrogen on the room-temperature tensile ductility;

FIG. 2 is a photograph showing the effect of various contents of carbon and nitrogen on the hot-workability of various alloy samples;

FIG. 3 is a graph showing the effect of manganese on the longitudinal tensile properties;

FIG. 4 represents anodic polarization curves for various steel compositions in a one normal sulfuric acid solution containing 0.5 moles of sodium chloride per liter;

FIG. 5 is a photograph showing the pitting characteristics of various stainless steel samples with varying contents of molybdenum;

FIG. 6 comprises photographs of four stainless steel samples each with varying molybdenum contents with respect to corrosion resistance; and

FIG. 7 is a graph showing the relationship of austenite and ferrite content on the hot workability and cold workability, with chromium equivalent (%) = %Cr + %Si + %Mo - 5Ni - 30 (%C+N).

As will be demonstrated and discussed in detail hereinafter the hot workability of the alloy is dependent upon restricting the combined carbon plus nitrogen contents. In addition, for this purpose, the composition with respect to the austenite and ferrite promoting elements must be balanced to achieve a chromium equivalent wherein the alloy has substantially equal amounts of ferrite and austenite. Hot workability is promoted by the presence of ferrite. Conversely hot workability is impaired by the presence of austenite. Austenite, however, promotes cold formability and thus must be present in the alloy for this purpose in combination with the ferrite necessary for hot workability to result in what is commonly termed a duplex alloy wherein the structure contains both austenite and ferrite. For purposes of corrosion resistance a minimum chromium content of 15 percent by weight is required. For this purpose, in combination with chromium, the alloy must contain molybdenum in an amount of at least 0.6 percent by weight; however, molybdenum must be restricted with regard to the maximum amount present as excessive amounts will have a detrimental effect on hot workability.

In accordance with the above the following constitutes a broad and preferred range of composition, in percent by weight, for a duplex stainless steel in accordance with the invention:

TABLE I

| Element              | Broad Range  | Preferred Range |
|----------------------|--------------|-----------------|
| Carbon               | 0.12 max.    | 0.10 max.       |
| Nitrogen             | 0.12 max.    | 0.06 max.       |
| Manganese            | 8 to 16      | 9 to 13         |
| Silicon              | 1.0 max.     | 0.5 max.        |
| Nickel               | 1.0 max.     | 0.5 max.        |
| Chromium             | 15 to 20     | 16 to 19        |
| Molybdenum           | 0.6 to 2.0   | 0.6 to 2.0      |
| Carbon + Nitrogen    | 0.06 to 0.14 | 0.08 to 0.13    |
| Chromium Equivalent* | 13.5 to 16.0 | 14.0 to 16.0    |

\*Chromium Equivalent (%) = %Cr + %Si + %Mo - %Ni - 30 (%C+N)

For applications of elevated temperature use requiring a high level of oxidation resistance the above-recited composition limits may be modified to provide a silicon content of up to about 3 percent by weight.

By way of specific examples and to establish the composition limits for the duplex stainless steel of the invention compositions presented in Table II were produced.

TABLE II

| Heat | Grade  | COMPOSITIONS OF EXPERIMENTAL ALLOYS |       |     |      |       |     | Mo   | N |
|------|--------|-------------------------------------|-------|-----|------|-------|-----|------|---|
|      |        | C                                   | Mn    | Si  | Ni   | Cr    |     |      |   |
| 1    | Duplex | .092                                | 5.87  | .30 | 0.29 | 17.03 | —   | .038 |   |
| 2    | do.    | .092                                | 7.89  | .29 | 0.38 | 16.96 | —   | .031 |   |
| 3    | do.    | .091                                | 9.70  | .29 | 0.30 | 16.88 | —   | .030 |   |
| 4    | do.    | .094                                | 11.67 | .27 | 0.29 | 16.79 | —   | .028 |   |
| 5    | do.    | .090                                | 9.42  | .38 | 0.34 | 17.55 | .24 | .027 |   |
| 6    | do.    | .090                                | 11.85 | .38 | 0.32 | 17.60 | .24 | .034 |   |
| 7    | do.    | .086                                | 9.31  | .51 | 0.33 | 17.21 | .25 | .037 |   |
| 8    | do.    | .084                                | 11.50 | .57 | 0.31 | 16.79 | .25 | .037 |   |
| 1E57 | do.    | .045                                | 11.89 | .30 | 0.33 | 17.23 | .25 | .034 |   |
| 1E59 | do.    | .069                                | 12.06 | .33 | 0.33 | 17.86 | .25 | .037 |   |
| 1E61 | do.    | .095                                | 12.13 | .34 | 0.33 | 17.45 | .25 | .041 |   |
| 1E62 | do.    | .095                                | 12.23 | .31 | 0.36 | 17.97 | .25 | .053 |   |
| 716  | do.    | .10                                 | 11.80 | .49 | 0.20 | 17.20 | .16 | .059 |   |
| 2314 | do.    | .084                                | 12.62 | .18 | 0.47 | 18.07 | .25 | .040 |   |
| 2309 | do.    | .084                                | 12.34 | .25 | 0.41 | 17.63 | .46 | .035 |   |
| 2310 | do.    | .082                                | 12.56 | .24 | 0.41 | 17.21 | .71 | .036 |   |
| 2311 | do.    | .081                                | 12.59 | .26 | 0.39 | 16.81 | .90 | .041 |   |
| 1C60 | T-430  | .072                                | 0.25  | .33 | —    | 16.64 | .23 | .034 |   |
| 2312 | T-434  | .052                                | 0.74  | .29 | 0.33 | 16.46 | .80 | .032 |   |
| 2313 | T-301  | .092                                | 1.19  | .28 | 7.32 | 17.72 | .27 | .033 |   |

To show the effect of carbon and nitrogen on the cold formability of the steel reference should be made to FIG. 1 of the drawings. As shown in FIG. 1, the designated alloys of TABLE II having varying carbon plus nitrogen contents were tested to determine room-temperature tensile ductility as a measure of cold formability. As may be seen from this FIGURE at carbon plus nitrogen contents of less than 0.06 percent elongation values, and thus cold formability, are poor; whereas, with increased carbon plus nitrogen content, and particularly carbon plus nitrogen contents of above about 0.08 percent, the elongation values drastically increase. Although cold formability continues to increase with carbon plus nitrogen contents above about 0.14 and 0.13 percent, at these high levels of carbon plus nitrogen the hot workability of the alloy is adversely affected. This is demonstrated by the photographs shown in FIG. 2. As may be seen with Heats 1E57, 1E59 and 1E61 of TABLE II the hot workability of the samples shown in the photograph of FIG. 2 was excellent; whereas, with Heats 1E62 and 716, which had carbon plus nitrogen contents of 0.148 and 0.159, respectively, samples were not satisfactory from the standpoint of hot workability. Consequently, it may be seen from this data that although carbon plus nitrogen contents in increasing amounts are beneficial from the standpoint of achieving cold formability, nevertheless they must be restricted to about 0.13 or 0.14 percent to permit satisfactory hot working of the stainless steel.

The presence of manganese within the range of 8 to 16 percent, and preferably 9 to 13 percent, is likewise necessary to achieve the desired cold formability. This effect of manganese is shown in FIG. 3. Specifically as may be seen from this FIGURE to achieve an elongation in 2 in. of 30 percent a manganese content of at least 8 percent is required as demonstrated by Heat 2 of TABLE II. In comparison, as may be seen from FIG. 3, with Heat 1 of TABLE II having a manganese content of 5.87 percent and an otherwise substantially identical composition to Heat No. 2 the elongation in 2 in. was approximately 18 percent as compared with approximately 30 percent for Heat No. 2. As may be seen from the elongation values presented in FIG. 3 for Heats 4, 6 and 8, all of which have manganese contents approaching about 12 percent, each of these alloys was characterized by excellent cold formability as measured by the percent elongation in 2 in.

The elements silicon and nickel are present only in normal residual amounts. However, silicon contents of up to about 3 percent may be desirable for elevated temperature applications requiring a high level of oxidation resistance.

Molybdenum is critical from the standpoint of providing suitable corrosion resistance for motor vehicle applications. Specifically, for this purpose at least about 0.6 percent molybdenum, and preferably about 1.0 percent molybdenum, is needed in the steel of the invention to produce corrosion resistance comparable to that of AISI Type 434, which is a standard stainless steel grade having minimum acceptable resistance to the corrosive effects of road deicing salts that are the primary corrosive environment for stainless steels used in motor vehicle applications. As may be seen from FIG. 4 potentiodynamic polarization tests in chloride-containing electrolyte indicate that about 0.90 percent molybdenum is required to produce pitting resistance comparable to Type 434. In the dip-dry tests, the re-

sults of which are shown in FIG. 5, it may be seen that with a residual molybdenum content of about 0.25 percent substantial pitting results; whereas, Type 434 is substantially free of pitting. It may be seen that with the samples constituting Heats 2310, 2311 having molybdenum contents of 0.71 and 0.90 percent, respectively, the pitting resistance improves over the low-molybdenum containing samples constituting Heats 2314 and 2309. Particularly with Heat 2311 having a 10 molybdenum content of 0.90 percent the sample shown in FIG. 5 of the drawing was completely free of pitting and equal to the Type 434 sample from this standpoint. As further evidence of the effect of molybdenum on corrosion resistance reference should be made to FIG. 15 6. As may be seen from these photographs of test samples that were in actual exposure on a passenger car driven in the Pittsburgh, Pennsylvania, area over the winter season 1969-1970 the corrosion resistance of the sample constituting Heat 2314 having residual molybdenum of about 0.25 percent was slightly poorer than the Type 434 sample; whereas, samples constituting Heats 2310 and 2311 having molybdenum contents of 0.71 and 0.90 percent, respectively, exhibited better 20 corrosion resistance than the Type 434 sample. As 25 would be expected from the above-reported data the sample constituting Heat 2311 having a molybdenum content of 0.90 percent showed essentially no corrosion and consequently was considerably superior to the Type 434 sample in this respect.

30 To obtain the optimum combination of hot workability and cold formability, it is necessary to balance the composition of the alloy with respect to the ferrite formers and austenite formers so as to produce substantially equal amounts of ferrite and austenite in the 35 structure of the alloy when annealed— typically within the range of 1,850° to 2,050°F. In this regard reference should be made to FIG. 7 of the drawings wherein it is shown that if the amount of the ferrite formers chromium, silicon, and molybdenum and the austenite promoters nickel, carbon and nitrogen are not properly balanced the corresponding balance of ferrite and austenite is not provided and consequently either hot workability or cold formability is impaired. More 40 specifically in this regard, if the composition balance with respect to the ferrite formers and austenite formers is such that less than 30 percent ferrite is present, e.g., chromium equivalent of less than 13.5 percent, hot workability is poor and inadequate for satisfactory 45 commercial production. If the composition balance is such that more than 65 percent ferrite is formed, e.g., chromium equivalent greater than 16.0 percent, the cold formability is decreased to a point where it is no longer superior to that of Type 434. From FIG. 7 it may 50 be seen, therefore, that the various austenite and ferrite 55 promoting elements in the composition must be carefully balanced to achieve the desired combination of hot workability and cold formability. In this regard, however, manganese is an exception in that the manganese content between 8 and 16 percent has no significant effect on the structure of the stainless steel from the standpoint of the austenite and ferrite content. 60 Manganese is important, however, as described above from the standpoint of its effect on room temperature ductility. Also, in maintaining a balance between the austenite and ferrite producing elements to achieve a chromium equivalent of 13.5 to 16 percent it is necessary that chromium be present in an amount of at least 65

15 percent from the standpoint of corrosion resistance. Amounts of chromium in excess of 20 percent, however, are not necessary for this purpose and merely unduly add to the cost of the alloy.

I claim:

1. A duplex stainless steel having good hot workability, cold formability and corrosion resistance consisting essentially of, in weight percent, carbon 0.12 max., nitrogen 0.12 max., manganese 8 to 16, silicon 3 max., nickel 1.0 max., chromium 15 to 20, molybdenum 0.6 to 2.0, carbon plus nitrogen 0.06 to 0.14 and balance iron, with a chromium equivalent of 13.5 to 16.0 in accordance with the formulae:

Chromium Equivalent, in percent = % chromium + % silicon + % molybdenum - % nickel - **30** (% carbon + % nitrogen),

to provide said steel with substantially equal amounts of ferrite and austenite after annealing within the range of 1,850° to 2,050°F, whereby a combination of both good hot workability and cold formability is achieved.

2. The steel of claim 1 having up to 10 percent silicon.

3. A duplex stainless steel having good hot workability, cold formability and corrosion resistance consisting essentially of, in weight percent, carbon 0.10 max., nitrogen 0.06 max., manganese 9 to 13, silicon 0.5 max., nickel 0.5 max., chromium 16 to 19, molybdenum 0.6 to 2.0, carbon plus nitrogen 0.08 to 0.13 and balance iron, with a chromium equivalent of 14.0 to 16.0 in accordance with the formulae:

Chromium Equivalent, in percent = % chromium + % silicon + % molybdenum - % nickel - **30** (% carbon + % nitrogen),

15 to provide said steel with substantially equal amounts of ferrite and austenite after annealing within the range of 1,850° to 2,050°F, whereby a combination of both good hot workability and cold formability is achieved.

\* \* \* \* \*

UNITED STATES PATENT OFFICE  
CERTIFICATE OF CORRECTION

Patent No. 3,861,908 Dated Jan. 21, 1975

Inventor(s) Jerome P. Bressanelli

It is certified that error appears in the above-identified patent and that said Letters Patent are hereby corrected as shown below:

Column 1, line 13, change "of" to --or--;

Column 6, claim 2, line 1, change "10" to --1.0--.

Signed and sealed this 17th day of June 1975.

(SEAL)

Attest:

RUTH C. MASON  
Attesting Officer

C. MARSHALL DANN  
Commissioner of Patents  
and Trademarks